

## UNITED STATES PATENT OFFICE

LOUIS LENFANT, OF PARIS, FRANCE, ASSIGNOR TO CARTIER, SOCIETE ANONYME, OF PARIS, FRANCE, A COMPANY OF FRANCE

## GOLD ALLOY

No Drawing. Application filed July 19, 1930, Serial No. 469,285, and in France June 14, 1930.

My invention has for its object an alloy containing, besides gold in the normal proportion of 750/1000 and other metals such as silver and copper, a certain quantity of 5 chromium.

Owing to this addition of chromium, this alloy possesses quite remarkable qualities which make its use particularly advantageous in jewelry.

10 In particular, this alloy is harder than the ordinary commercial metals or alloys, so that it can be used in thinner form. Furthermore, the presence of copper gives the alloy a redder, warmer shade than that of ordinary 15 white gold. Lastly, this alloy does not harden when hammered or drawn in the cold state and it can be rolled to one tenth of its original thickness without annealing, which is very important for jewelry. Of course it 20 is perfectly ductile and can easily be stamped.

By way of example optimum limits for the proportion of chromium can be indicated as ranging from 0.001 to 0.025. The alloy would then have the following composition: 25 gold: 750 per thousand, chromium: from 1 to 25 per thousand, silver and copper: the remainder.

As a result of my experiments I have found out that the percentage of copper should 30 preferably be higher than that of silver, the proportion being, for instance:

$$\frac{\text{quantity of copper}}{\text{quantity of silver}} = 1,4$$

35 The following composition of the alloy may be given by way of example:

|          | Per<br>thousand |
|----------|-----------------|
| Gold     | 750             |
| Copper   | 140             |
| Silver   | 100             |
| Chromium | 10              |

but it should be well understood that this 45 indication is not limitative.

What I claim is:—

A gold alloy intended for jewelry having the following composition:

|          | Per cent |
|----------|----------|
| Gold     | 75       |
| Copper   | 14       |
| Silver   | 10       |
| Chromium | 1        |

In testimony whereof I have signed this specification.

LOUIS LENFANT.

60

65

70

75

80

85

90